# EUROPEAN PATENT APPLICATION

(11) **EP 4 349 184 A1**
(43) Date of publication of application: **10.04.2024**
(21) Application number: 22814950.6
(22) Date of filing: 05.05.2022
(51) Int. Cl.: A24B 15/167, A24F 40/70

(54) **HEAT-NOT-BURN CIGARETTE, PLANT FIRMWARE, AND PREPARATION METHOD THEREFOR**

(30) Priority: 31.05.2021 CN 202110598615
(71) Applicant: Shanghai Huabao Biology Technology Co., Ltd., Shanghai 201800 (CN); Jishou Huajin Bio-Technology Co., Ltd., Jishou, Hunan 416000 (CN)
(72) Inventor: XU, Xiaodong, Shanghai 201800 (CN); SHEN, Li, Shanghai 201800 (CN); LIANG, Jiasheng, Shanghai 201800 (CN); YING, Yu, Shanghai 201800 (CN); GAO, Guoying, Shanghai 201800 (CN); FU, Yuanfeng, Shanghai 201800 (CN); GAO, Xu, Shanghai 201800 (CN)
(74) Representative: Huang, Liwei
(86) International application number: PCT/CN2022/090919
(87) International publication number: WO 2022/252903

(57) **Abstract**

The application claims a heat-not-burn cigarette, plant part, and preparation method thereof. The preparation method of the plant part comprises the following steps: Mixing the powder and water used to make plant part to form a wet material to be extruded; Molding the wet material to form a semi-finished plant part; Baking the semi-finished plant part to form the plant part, wherein the elastic modulus of the plant part after drying is within 7-20.

## Description

### Cross-Reference to Related Application

This application claims the priority of the Chinese patent application No. 2021105986159, entitled "heat-not-burn cigarette, plant part, and production method thereof", filed with the China National Intellectual Property Administration on May 31, 2021, the whole contents of which are incorporated by reference in this application.

### Technical Field

The application relates to the field of the heat-not-burn cigarette, in particular to the heat-not-burn cigarette, plant part, and preparation method thereof.

### Background

At present, the composite filter rod commonly used in the tobacco industry refers to an object composed of two or more small sections of different varieties of filter rods connected end to end, and then wrapped by the same sheet of wrap paper, and then compounded on the composite forming machine.

By adding a cooling plant part between the smoke section and the filter rod, the heat-not-burn cigarette section can prevent excessive heat from transferring to the end of the filter rod, so as to ensure that the user is not burned. The plant part is also usually used as a section of the filter rod, that is, the filter rod in the heat-not-burn cigarette is more of a composite filter rod with plant part.

In the rolling process of the heat-not-burn cigarette, in addition to the roundness and circumference of the plant part, it also requires a certain hardness and elasticity of the plant part. Because the plant part usually needs to be cut into a predetermined length after production. For the relevant technology, it is easy to have abnormal phenomena such as chip dropping, knife breaking, and knife sticking during cutting. In addition, during the rolling process of the filter rod and smoking material, the plant part needs to pass through a press wheel, which exerts a certain pressure on the plant part and moves a predetermined distance. At this time, if the plant part is too hard and lacks a certain elasticity, the plant part may break, and then affect the quality of the final composite filter rod.

In addition, after the processing of the plant part with the related technology, in order to ensure the taste and forming effect, the plant part will reserve excessive water. Besides, this is bound to affect the elasticity of the plant part, so it will affect the pass rate of the plant part on the machine, that is, the success rate of plant part production.

### Summary

An advantage of the application is that, for example, the heat-not-burn cigarette, plant part, and preparation method thereof are provided, wherein the plant part prepared by the preparation method of the application has a high pass rate on the machine.

Another advantage of the application is, for example, the heat-not-burn cigarette, plant part, and preparation method thereof are provided, wherein the plant part prepared by the preparation method of the application has good hardness and predetermined elasticity, thereby preventing the plant part from irreversible deformation under pressure.

Another advantage of the application is, for example, the heat-not-burn cigarette, plant part, and preparation method thereof are provided, wherein the plant part prepared by the preparation method of the application does not have any abnormal phenomena such as chip dropping, knife breaking and knife sticking during the making process.

An advantage of the application is, for example, a method for making plant part is provided, which may comprise the following steps:
Mixing the powder and water used to make plant part to form a wet material to be extruded;
Molding the wet material to form a semi-finished plant part; and
Baking the semi-finished plant part to form the plant part, wherein the elastic modulus of the plant part after drying is within 7-20.

According to an embodiment of the application, the preparation method of the plant part may comprise the following steps:
Determining the moisture content of the wet material, and controlling the moisture content of the wet material between 25% and 35% (mass fraction).

According to an embodiment of the application, the mass fraction of liquid water can be 46%-52%, of which the mass fraction of powder can be 45%-51%.

According to an embodiment of the application, the value of the elastic modulus of the dried plant part may be within 7-10 or 12-20.

According to an embodiment of the application, the value of the elastic modulus of the semi-finished dried plant part may be within 7-10 or 12-20.

According to an embodiment of the application, for the semi-finished plant part whose molded water content is controlled within 25%-35%, the plasticity index of the wet material is determined and controlled within 0.45-0.7.

According to an embodiment of the application, the plasticity index of the wet material before molding may be within 0.6-0.7 or 0.45-0.55.

According to an embodiment of the application, when baking the semi-finished plant part, the baking temperature is 90°C-110°C, and the baking time is 30-90min.

According to an embodiment of the application, the preparation method of the plant part comprises mixing plant raw material powder of 3-5 parts by weight, blinder of 4-6 parts by weight, and water of 4-6 parts by weight to make a wet material to be extruded.

According to an embodiment of the application, the powder for making the plant part also comprises a smoking agent of 4-6 parts by weight.

According to an embodiment of the application, the plant raw material powder is at least one selected from the tobacco leaf powder, herbal plant powder, or woody plant powder.

According to an embodiment of the application, the smoking agent is selected from at least one of the food-grade glycerin and propylene glycol.

According to an embodiment of the application, the binder is one or more selected from food-grade starch, microcrystalline cellulose, CMC-Na, etc.

To achieve at least one of the above advantages of the present application, the application provides plant part that can be produced by the preparation method of the plant part.

The application provides a heat-not-burn cigarette. The heat-not-burn cigarette may comprise a smoking section and a filter rod section connecting to one end of the smoking section. The filter rod may comprise a filter rod body and the plant part as mentioned above, two ends of which are respectively connected to the filter rod body and the smoking section. The heat-not-burn cigarette provided in the application achieves at least one of the advantages mentioned above.

According to an embodiment of the application, the plant part may be made of a paste mixture formed by plant raw material powder of 3-5 parts by weight, binder of 4-6 parts by weight, and water of 4-6 parts by weight.

### Brief Description of the Drawings

FIG. 1 shows a schematic diagram of a heat-not-burn cigarette in the application.
FIG. 2 shows a flow diagram of the method for preparing the heat-not-burn cigarette in the application.

### Description of Embodiments

The following description is intended to expose the application so that a person skilled in the art can implement it. The preferred embodiments described below are examples only, and those skilled in the art may think of other obvious variations. The basic principles of the application defined in the following description, may be applied to other embodiments, variants, improvements, equivalents, and other technical solutions that do not deviate from the spirit and scope of the application.

It should be understood by a person skilled in the art that, in the disclosure of this application, the terms "vertical", "horizontal", "up", "down", "front", "back", "left", "right", "vertical", "horizontal", "top", "bottom", "inside", "outside", etc. indicate orientation or position relationships based on the orientation or position relationships shown in the drawings. They are intended only to facilitate the description of this application and to simplify the description and do not indicate or imply that the device or element referred to must have a particular orientation, structure, and operation in a particular orientation. Therefore, the above terms are not to be construed as a limitation of the application.

It is understandable that the term "one" shall be understood as "at least one" or "one or more", i.e., in one embodiment, the number of an element may be one, while in another embodiment the number of the element may be multiple, and the term "one" shall not be understood as a limitation on the number.

With reference to FIG.1, the heat-not-burn cigarette 100 according to the embodiment of the application is described in detail below, wherein the heat-not-burn cigarette 100 may comprise a smoking section 10 and a filter rod section 20 connecting to one end of the smoking section 10. The filter rod section 20 may comprise a filter rod body 21 and a plant part 22, and both ends of the plant part 22 are connected to the filter rod body 21 and the smoking section 10 respectively.

The plant part 22 can be made by powder and water when preparing. The powder for preparing the plant part 22 may comprise the plant raw material powder of 3-5 parts by weight, and blinder of 4-6 weight parts by weight. Preferably, the powder may also comprise the smoking agent of 4-6 parts by weight. In addition, the cross-section shape of the plant part 22 can usually be circular, and the plant part 22 can form air holes through both ends of the plant part 22 after production.

It is precisely because of the shape requirements of the plant part 22 itself that the plant part 22 is easy to break in the production process.

It is worth mentioning that the plant raw material powder may be at least one selected from the tobacco leaf powder, herbal plant powder, or woody plant powder.

The herbs may be herbs with a certain aroma, a certain medicinal value, or a certain physiological satisfaction, including but not limited to tobacco leaf, orange peel, licorice, pueraria, basil, mint, lavender, and lemongrass. The woody plant may be a woody plant with a certain aroma, a certain medicinal value, or a certain physiological satisfaction, including but not limited to honeysuckle.

Optionally, the smoking agent may be implemented as at least one of the food-grade glycerin and propylene glycol.

The binder may be a hot melt plant powder. The binder can be used to knead the tobacco raw material powder, the smoking agent, and the binder. The binder may be implemented as one or more selected from food-grade starch, microcrystalline cellulose, CMC-Na, etc.

In addition, the plant part may be prepared in the following manner:
S3001: Mixing powder and water for making the plant part; Preferably, the powder can be the plant raw material powder, binder, and smoking agent to make a wet material to be extruded;
S3002: Molding the wet material to form a semi-finished plant part; and
S3003: Baking the semi-finished plant part to form the plant part, wherein the elastic modulus of the plant part after drying is within 7-20.

In one embodiment, the plant part may be prepared in the following manner:
Mixing the plant raw material powder of 3-5 parts by weight, binder of 4-6 parts by weight, and water of 4-6 parts by weight to make a wet material to be extruded;
Molding the wet material to form a semi-finished plant part; and
Baking the semi-finished plant part to form the plant part, wherein the moisture content of the wet material in the step S3001 is controlled between 25% and 35% (mass fraction).

Preferably, the powder for making the plant part may also comprise the smoking agent of 4-6 parts by weight.

In addition, in the step S3001, the mass fraction of the liquid is 46%-52%, and the mass fraction of the powder is 45%-51%. Preferably, the moisture content of the wet material is controlled at 25%-30% or 30%-35%. If the moisture content is higher than this range, the final product will be soft in texture and easy to absorb moisture resulting in reduced quality; if it is lower than this range, the final product will be dry in texture and prone to cracks in appearance. In addition, the value of the elastic modulus of the dried plant part is within 7-20. As a preference, the value of the elastic modulus of the dried plant part is within 7-10 or 12-20.

That is, the plant part production method may also comprise determining the water content of the wet material. It is understood by those skilled in the art that the moisture content of the wet material can be determined by a rapid moisture meter.

In addition, the elastic modulus of the plant part can be detected by an elastic modulus detector. The detection methods may include but are not limited to, stretching methods. For example, the equipment for measuring the elastic modulus can be a computer-controlled single-column tension tester. When testing, the plant part can be contacted by the sensor based on the mechanical properties and related physical parameters under a compression state. The pre-installed software of the equipment can calculate the elastic modulus value of the sample to be measured in real-time.

Also, as a preference, the plasticity index of the wet material before molding shall be controlled at 0.45-07. Preferably, the plasticity index of the wet material before molding is within 0.6 and 0.7 or 0.45 and 0.55. If the plasticity index is higher than this range, the final product will have poor elasticity and will be easy to cause cutting chips or even a broken knife. If the plasticity index is lower than this range, the final product is sticky and easy to stick. It is understood by those skilled in the art that the plasticity index can be measured quickly by the plasticity tester.

As preferred, in the step S3003, when baking the semi-finished plant part, the baking temperature is 90°C-110°C, and the baking time is 30min-90min.

It is understandable that by controlling the moisture content of the wet material, the elastic modulus of the semi-finished plant part after drying, the plasticity index of the semi-finished plant part during molding, and the temperature and time during baking, the plant part finally formed has a good passing rate on the machine. In this way, not only ensures the elasticity of the plant part and prevents the plant part from irreversible deformation when it is under pressure, but also cannot occur in the plant part production process, such as chip dropping, knife breaking, and knife sticking. After evaluation, the pass rate of the plant part prepared by the method proposed in the patent can be increased to 70%-85% after compositing on the machine.

| | Whether controlling the ratio of liquid and powder | Whether controllin g the water content | Whether controlling the plasticity index | Whether controlling the baking time and temperature | Whether controlling the elastic modulus of finished products | Rolling of finished products on the machine |
|---|---|---|---|---|---|---|
| Comparative example I | The proportion of liquid mass fraction is 58%, and the proportion of powder mass fraction is 42% | The moisture content of mud is 35% | The plasticity index is 0.4 | The temperature is 110°C and the time is 80min | The elastic modulus of the finished product is 10 | Chip dropping, knife breaking in cutting; plant part is easy to crack |
| Embodiment I | Controlling the proportion of liquid mass in 46-52% and controlling the proportion of powder mass in 45-51% | Controllin g the moisture content of mud in 25-30% | Controllin g the plasticity index in 0.6-0.7 | Controlling the temperature at 100-110°C and controlling time at 70-90min | Controlling the elastic modulus of the finished product in 12-20 | Obvious decrease in chip dropping and knife breaking. No breaking of the plant part |
| Comparative example II | The proportion of liquid mass fraction is 40%, and the proportion of powder mass fraction is 60% | The moisture content of mud is 27% | The plasticity index is 0.65 | The temperature is 105°C and the time is 40min | The elastic modulus of the finished product is 14 | Knife sticking in cutting; plant part is easy to crack |
| Embodiment II | Controlling the proportion of liquid mass in 44-48% and controlling the proportion of powder mass in 48-54% | Controllin g the moisture content of mud in 30-35% | Controllin g the plasticity index in 0.45-0.55 | Controlling the temperature at 90-105°C and controlling time at 30-50min | Controlling the elastic modulus of the finished product in 7-10 | Obvious decrease in knife sticking dropping. No breaking of the plant part |

It should be understood by those skilled in the art that the above description and embodiments of the application shown in the drawings are examples only and do not limit the application. The advantages of the application have been fully and effectively realized. The functional and structural principles of the application have been demonstrated and illustrated in embodiments, and the embodiments of the application may be subject to any distortion or modification without departure from the principles.

### Industrial Applicability

The application claims a heat-not-burn cigarette, plant part, and preparation method thereof. The preparation method of the plant part comprises the following steps: Mixing the powder and water used to make plant part to form a wet material to be extruded; Molding the wet material to form a semi-finished plant part; Baking the semi-finished plant part to form the plant part, wherein the elastic modulus of the plant part after drying is within 7-20.

In addition, it is understandable that the heat-not-burn cigarette, plant part, and preparation method of the application are reproducible and can be applied in a variety of applications. For example, the preparation method of the heat-not-burn cigarette and plant part of the application may be applied to the preparation of the heat-not-burn cigarette and plant part.

## Claims

1. A preparation method of a plant part, wherein the preparation method of the plant part comprises the following steps:
Mixing the powder and water used to make plant part to form a wet material to be extruded;
Molding the wet material to form a semi-finished plant part; and
Baking the semi-finished plant part to form the plant part, wherein the elastic modulus of the plant part after baking is within 7-20.

2. The preparation method of the plant part according to claim 1, wherein the preparation method of the plant part comprises the following steps:
Determining the moisture content of the wet material, and controlling the moisture content of the wet material between 25% and 35% (mass fraction).

3. The preparation method of the plant part according to claim 1 or 2, wherein the mass fraction of liquid water is 46%-52%, and the mass fraction of powders is 45%-51%.

4. The preparation method of the plant part according to any one of the claims 1-3, wherein the value of the elastic modulus of the baked plant part is within 7-10 or 12-20.

5. The preparation method of the plant part according to any one of the claims 2-4, wherein the preparation method of the plant part comprises the following steps:
molding the semi-finished plant part whose water content is controlled within 25%-35%, the plasticity index of the wet material is determined and controlled within 0.45-0.7.

6. The preparation method of the plant part according to claim 5, wherein the plasticity index of the wet material before molding is within 0.6-0.7 or 0.45-0.55.

7. The preparation method of the plant part according to any one of the claims 1-6, wherein when baking the semi-finished plant part, the baking temperature is 90°C-110°C, and the baking time is 30min-90min.

8. The preparation method of the plant part according to any one of the claims 1-7, wherein the preparation method of the plant part comprises mixing plant raw material powders of 3-5 parts by weight, binder of 4-6 parts by weight, and water of 4-6 parts by weight to form a wet material to be extruded.

9. The preparation method of the plant part according to any one of the claims 1-8, wherein the powders for making the plant part also comprises a smoking agent of 4-6 parts by weight.

10. The preparation method of the plant part according to claim 8, wherein the plant raw material powders are at least one selected from the tobacco leaf powder, herbal plant powder, or woody plant powder.

11. The preparation method of the plant part according to claim 9, wherein the smoking agent is at least one selected from food-grade glycerin and propylene glycol.

12. The preparation method of the plant part according to claim 8 or 10, wherein the binder is one or more selected from food-grade starch, microcrystalline cellulose, CMC-Na, etc.

13. A plant part, wherein the plant part is produced according to the preparation method of the plant part in any of above claims 1-12.

14. A heat-not-burn cigarette, wherein the heat-not-burn cigarette comprises a smoking section, and a filter rod section connecting to one end of the smoking section, the filter rod section comprises a filter rod body and a plant part according to claim 13, and two ends of the plant part are connected to the filter rod body and the smoking section respectively.

15. The heat-not-burn cigarette according to claim 14, wherein the plant part is made of a paste mixture formed by plant raw material powders of 3-5 parts by weight, binder of 4-6 parts by weight, and water of 4-6 parts by weight.
